

# United States Patent [19]

Ueda

[11] Patent Number: 4,939,053

[45] Date of Patent: Jul. 3, 1990

[54] PHOTOSENSITIVE MEMBER INCLUDING AZO COMPOUND

[75] Inventor: Hideaki Ueda, Osaka, Japan

[73] Assignee: Minolta Camera Kabushiki Kaisha, Osaka, Japan

[21] Appl. No.: 154,385

[22] Filed: Feb. 10, 1988

[30] Foreign Application Priority Data

Feb. 12, 1987 [JP] Japan 62-30481

[51] Int. Cl.<sup>5</sup> G03G 5/06; G03G 5/14

[52] U.S. Cl. 430/58; 430/75; 430/77; 430/72; 430/73; 430/78; 430/76; 430/70; 430/79; 534/738; 534/755; 534/757; 534/761; 584/772

[58] Field of Search 534/755, 757, 758, 738, 534/761, 772; 430/58, 59, 72, 73, 76, 78, 75, 77

[56] References Cited

U.S. PATENT DOCUMENTS

- |           |         |                  |           |
|-----------|---------|------------------|-----------|
| 4,032,339 | 6/1977  | Grushkin et al.  | 96/1.5    |
| 4,062,854 | 12/1977 | Grushkin         | 544/211 X |
| 4,123,270 | 10/1978 | Heil et al.      | 430/72 X  |
| 4,272,598 | 6/1981  | Sasaki et al.    | 430/72    |
| 4,396,695 | 8/1983  | Dimmler et al.   | 430/59    |
| 4,396,696 | 8/1983  | Nagasaki et al.  | 430/78    |
| 4,399,206 | 8/1983  | Katagiri et al.  | 430/58    |
| 4,419,428 | 12/1983 | Katagiri et al.  | 430/77    |
| 4,426,432 | 1/1984  | Sawada et al.    | 534/761 X |
| 4,515,881 | 5/1985  | Sawada et al.    | 430/58    |
| 4,533,613 | 8/1985  | Kawamura et al.  | 430/78    |
| 4,537,847 | 8/1985  | Takahashi et al. | 430/58    |
| 4,540,651 | 9/1985  | Fujimaki et al.  | 430/72    |
| 4,554,231 | 11/1985 | Ishikawa et al.  | 430/59    |
| 4,582,771 | 4/1986  | Ohta et al.      | 534/738 X |
| 4,631,242 | 12/1986 | Emoto et al.     | 430/58    |
| 4,647,520 | 3/1987  | Watanabe et al.  | 534/761 X |
| 4,663,442 | 5/1987  | Ohta             | 534/738 X |
| 4,672,149 | 6/1987  | Yoshikawa et al. | 534/738 X |
| 4,687,721 | 8/1987  | Emoto et al.     | 430/58    |
| 4,702,982 | 10/1987 | Matsumoto et al. | 430/72    |
| 4,716,220 | 12/1987 | Tsutsui          | 534/738   |
| 4,743,523 | 5/1988  | Yamashita et al. | 534/832 X |

4,760,003 7/1988 Matsumoto et al. 534/738 X  
4,820,600 4/1989 Akasaki et al. 430/68

FOREIGN PATENT DOCUMENTS

- |           |         |       |           |
|-----------|---------|-------|-----------|
| 54-22834  | 2/1979  | Japan | 430/58    |
| 55-117151 | 9/1980  | Japan | 534/738 X |
| 59-214034 | 12/1984 | Japan | 430/58    |
| 60-19152  | 1/1985  | Japan | 430/58    |
| 60-121451 | 6/1985  | Japan | 534/761   |
| 61-272755 | 12/1986 | Japan | 430/58    |
| 62-55662  | 11/1987 | Japan | 430/58    |
| 62-55786  | 11/1987 | Japan | 430/58    |
| 62-58505  | 12/1987 | Japan | 430/58    |
| 62-59299  | 12/1987 | Japan | 430/58    |

Primary Examiner—Floyd D. Higel

Attorney, Agent, or Firm—Burns, Doane, Swecker & Mathis

[57]

ABSTRACT

The present invention relates to a photosensitive member containing a specific azo compound for a charge generating agent, which is improved in photosensitive properties, in particular, sensitivity. The specific azo compound is represented by the formula (1):



wherein A represents an aromatic hydrocarbon or a heterocyclic ring; R<sub>1</sub> and R<sub>2</sub> independently represent a hydrogen, a halogen atom, or an alkyl, aralkyl, aryl, condensed polycyclic ring or condensed heterocyclic ring; or R<sub>1</sub> and R<sub>2</sub> combinedly form a cyclic ring; n represents an integer from 1 to 4.

11 Claims, No Drawings

## PHOTOSENSITIVE MEMBER INCLUDING AZO COMPOUND

### BACKGROUND OF THE INVENTION

This invention relates to a photosensitive member containing a new azo dye.

Known photosensitive materials for forming a photosensitive member, include inorganic photoconductive materials such as selenium, cadmium sulfide or zinc oxide.

These photosensitive materials have many advantages such as low loss of charges in the dark, the electrical charge can be dissipated fast with irradiation of light and the like. However, they have disadvantages. For example, a photosensitive member based on selenium is difficult to produce, has high production costs and is difficult to handle due to inadequate resistivity to heat or mechanical impact. A photosensitive member based on cadmium sulfide or zinc oxide has defects such as an unstable sensitivity in a highly humid environment and loss of stability with time because of the deterioration of dyestuffs, added as a sensitizer, by corona charge and fading with exposure.

Many kinds of organic photoconductive materials such as polyvinylcarbazole and the like have been proposed. These organic photoconductive materials have superior film forming properties, are light in weight, etc., but inferior in sensitivity, durability and environmental stability compared to the aforementioned inorganic photoconductive materials.

Various studies and developments have been in progress to overcome the above noted defects and problems. Function-divided photosensitive members of a laminated or a dispersed type have been proposed, in which the charge generating function and charge transporting function are divided by different layers or different dispersed materials. The function-divided photosensitive member can be a highly efficient photosensitive member in electrophotographic properties such as chargeability, sensitivity, residual potential, durability to copy and repetition, because most adequate materials can be selected from various materials. Further, function-divided photosensitive members have high productivity and low costs, since it can be prepared by coating, and adequately selected charge generating materials can freely control a region of photosensitive wavelength. Illustrative examples of such charge generating materials are organic pigments or dyes such as phthalocyanine pigment, cyanine pigment, polycyclic quinone pigment, perylene pigment, Perinone pigment, indigo dye, thioindigo dye, squarain compounds, etc., and inorganic materials such as selenium, selenium-arsenic, selenium-tellurium, cadmium sulfide, zinc oxide, amorphous silicon, etc.

However, such photosensitive members, which satisfy general static properties, are not produced easily, and the sensitivity can be further improved.

### SUMMARY OF THE INVENTION

The object of the invention is to provide a photosensitive member having excellent general static properties, in particular, sensitivity.

The present invention relates to a photosensitive member wherein a photosensitive layer containing an azo pigment represented by the general formula(I) is formed on an electroconductive substrate;



wherein A represents an aromatic hydrocarbon group or a heterocyclic group, which may be bonded through a bonding group; R<sub>1</sub> and R<sub>2</sub> independently represent any of hydrogen, halogen atom, or an alkyl group, an aralkyl group, an aryl group, a condensed polycyclic group or a condensed heterocyclic group, any of which may have a substituent; R<sub>1</sub> and R<sub>2</sub> may combinedly form a cyclic ring; n represents an integer of 1-4.

### DETAILED DESCRIPTION OF THE INVENTION

25 The present invention provides a photosensitive member having excellent electrophotographic properties, in particular, sensitivity.

The present invention accomplished the above object by introduction of a specific azo pigment as a charge generating material into a photosensitive member.

30 A photosensitive member provided according to the present invention contains a specific azo compound represented by the following formula (I)



wherein A represents an aromatic hydrocarbon group or a heterocyclic group, which may be bonded through a bonding group; R<sub>1</sub> and R<sub>2</sub> independently represent any of hydrogen, halogen atom, or an alkyl group, an aralkyl group, an aryl group, a condensed polycyclic group or a condensed heterocyclic group, any of which may have a substituent; R<sub>1</sub> and R<sub>2</sub> may combinedly form a cyclic ring; n represents an integer of 1-4.

45 A compound of the invention represented by the general formula (I) can be synthesized according to a known method. For example an N-amino compound represented by the general formula (II);



55 wherein A and n are the same as above, may be reacted with sodium nitrite in hydrochloric acid to form an azo compound, which may be coupled with an appropriate coupler represented by the following general formula (III) in the presence of alkali,



5

-continued



10.

5  
10  
11.12.  
20  
2513.  
30  
3514.  
40  
45

6

-continued

17.



18.



19.



20.

15.  
50  
55

21.

16.  
60  
65

22.

-continued



-continued



Preferred couplers above are, in particular, shown by (2), (7) (10), (11), (12), (14), (16), (26) and (27).  
A method of production of a photosensitive member comprising an azo pigment represented by the general formula (I) with the above coupler component (1) is shown below, and other azo pigments with the other coupler components can be similarly synthesized according to the method of synthesis as discussed in detail below.

#### EXAMPLE OF SYNTHESIS 1

3,3'-Dichlorobenzidine (2.53 g, 0.01 mole) was dispersed in hydrochloric acid (100 ml). The dispersion was stirred and cooled to 5° C., followed by the addition of an aqueous solution of sodium nitrite (1.4 g) in water (20 ml). Further, the mixture was stirred, as it cooled, for one hour, and then filtered. Borofluoric acid (10 g) was added to the filtrate and then crystallized. The obtained crystals were filtered to give 3,3'-dichlorobenzidine tetrafluoroborate.

Then, the resultant diazonium salt (3.49 g, 0.01 mole) and the coupling agent (6.32 g) represented by the above coupling component (1) were dissolved in N-methylpyrrolidone (300 ml), to which a solution of sodium acetate (5) dissolved in 100 ml of water is added at 10°-20° C. for about 30 minutes. After the addition, the solution was further stirred at the room temperature for 3.5 hours to filtrate the deposited crystals.

The resultant crystals were dispersed in 1:1 mixture of DMF, and the solution was stirred at room temperature for 3.5 hours, followed by filtration of the crystals. This operation was repeated two more times. Then, the crystals were washed with water and dried to produce 7.1 g (78.3% of yield) of disazo pigment. Violet-red crystals were obtained.

| 28. | elemental analysis |       |       |
|-----|--------------------|-------|-------|
|     | element            | C     | H     |
| 60  | found              | 66.19 | 3.01  |
|     | calcd.             | 66.15 | 3.09  |
|     |                    | 12.40 | 12.35 |

Components of A in the general formula (I) of the invention were shown below with no significance with respect to restricting the embodiments.



-continued



-continued



wherein X and R represent a halogen atom, a hydrogen, an alkyl group or an alkoxy group respectively, and n is an integer of 0 or 1.

A photosensitive member of the invention has a photosensitive layer comprising one or more azo pigments represented by the aforementioned general formula (I). A photosensitive member, various types of which are known, may be any type in the invention. For example, a photosensitive member of the invention may be a monolayer type in which a photosensitive layer is formed on a substrate by dispersing azo pigments in a resin binder or a charge transporting medium, or a laminated type in which first a charge generating layer containing mainly an azo pigment is formed on a substrate and then a charge transporting layer is formed on the charge generating layer. An azo pigment of the invention functions as a photoconductive material and generates charges with very high efficiency by absorbing light. The generated charges may be transported with an azo pigment as a medium, but more effectively with a charge transporting material as a medium.

In order to form a photosensitive member of a monolayer type, fine particles of an azo pigment are dispersed in a resin solution or a solution containing a charge transporting compound and resin, which is spray dried on an electrically conductive substrate. The thickness of the photosensitive layer is 3-30  $\mu\text{m}$ , preferably 5-20  $\mu\text{m}$ . The sensitivity is poor if the azo pigment is used in an insufficient quantity, whereas if used to an excess the chargeability is poor and the mechanical strength of the photosensitive layer is inadequate. The amount of an azo pigment is within the range of 0.01-2 parts by weight, preferably, 0.2-1.2 parts by weight on the basis of one part by weight of resin. If a charge transporting material is used such as polyvinylcarbazole, which is capable of being used as a binder itself, an additional amount of an azo pigment is also used preferably 0.01-0.5 parts by weight on the basis of one part by weight of charge transporting materials.

In order to form a photosensitive member of the laminate type, an azo pigment is deposited in a vacuum on a substrate, dissolved in an amine solvent to apply onto a substrate or dissolved in an application solution containing an azo pigment and, if necessary, binder resin dissolved in an appropriate solvent to apply onto a substrate to be dried. Then, a solution containing a charge transporting material and a binder is applied onto the charge generating layer. The thickness of the azo pigment-containing layer, as a charge generating layer, is 4  $\mu\text{m}$  or less, preferably, 2  $\mu\text{m}$  or less. It is suitable that the charge-transporting layer has a thickness in the range 3-30  $\mu\text{m}$ , preferably 5-20  $\mu\text{m}$ , and the proportion of charge transporting materials in the

charge-transporting layer is 0.2-2 parts by weight, preferably 0.3-1.3 parts by weight on the basis of one part by weight of the binder. There is no need to use a binder when the charge-transporting material is a high-polymer which is capable of serving as a binder itself.

A photosensitive member of the present invention permits, in combination with the binder, the use of a plasticizer, such as halogenated paraffin, polybiphenyl chloride, dimethyl naphthalene, dibutyl phthalate or O-terphenyl, the use of an electron-attractive sensitizer, such as chloranyl, tetracyanoethylene, 2,4,7-trinitrofluorenone, 5,6-dicyanobenzoquinone, tetracyanoquinodimethane, tetrachlorphthalic anhydride, or 3,5-dinitrobenzoic acid, and the use of a sensitizer, such as methyl violet, rhodamine B, cyanine dye, pyrlyium salt, and thiapyrylium salt. Applicable as a binder in the practice of this invention are any of thermoplastic resins and thermosetting resins which are publicly known to be electrically insulative and any of the photocuring resins and photoconductive resins.

Some examples of suitable binders are thermoplastic resins such as saturated polyester, polyamide, acrylic, ethylene-vinyl acetate copolymer, ion cross-linked olefin copolymer (ionomer), styrene-butadiene block copolymer, polycarbonate, vinyl chloride-vinyl acetate copolymer, cellulose ester, polyimide, styrol, etc., and thermosetting resins such as, epoxy, urethane, silicone, phenolic, melamine, xylene, alkyd, thermosetting acrylic, etc., and photocuring resins, and photoconductive resins such as poly-N-vinyl carbazole, polyvinyl pyrene, polyvinyl authracene, etc., all named without any significance of restricting the use to them. Any of these resins can be used singly or in combination with other resins. It is desirable for any of these electrically insulative resins to have a volume resistance of  $1 \times 10^{12} \Omega \cdot \text{cm}$  or more when measured singly.

Illustrative examples of charge transporting materials are hydrazone compounds, pyrazoline compounds, styryl compounds, triphenylmethane compounds, oxadiazol compounds, carbazole compounds, stilbene compounds, enamine compounds, oxazole compounds, triphenylamine compounds, tetraphenylbenzidine, azine compounds and so on, including carbazole, N-ethylcarbazole, N-vinylcarbazole, N-phenylcarbazole, tetracene, chrysene, pyrene, perylene, 2-phenylnaphthalene, azapyrene, 2,3-benzochrysene, 3,4-benzopyrene, fluorene, 1,2-benzofluorene, 4-(2-fluorenylazo)-resorcinol, 2-p-anisolaminofluorene, p-diethylaminoazobenzene, cadion, N,N-dimethyl-p-phenylazoaniline, p-(dimethylamino)stilbene, 1,4-bis(2-methylstyryl)benzene, 9-(4-diethylaminostyryl)anthracene, 2,5-bis(4-diethylaminophenyl)-1,3,5-oxadiazole,

1-phenyl-3-(p-diethylaminostyryl)-5-(p-diethylamino-phenyl)pylazoline, 1-phenyl-3-phenyl-5-pylazolone, 2-(m-naphthyl)-3-phenyloxazole, 2-(p-diethylaminostyryl)-6-diethylaminobenzoxazazole, 2-(p-diethylaminostyryl)-6-diethylaminobenzothiazazole, bis(4-diethylamino-2-methylphenyl)phenylmethane, 1,1-bis(4-N,N-diethylamino-2-ethylphenyl)heptane, N,N-diphenylhydrazino-3-methylidene-10-ethylphenoxazine, N,N-diphenylhydrazino-3-methylidene-10-ethylphenothiazine, 1,1,2,2-tetrakis-(4-N,N-diethylamino-2-ethylphenyl)ethane, p-diethylaminobenzaldehyde-N,N-diphenylhydrazone, p-diphenylaminobenzaldehyde-N,N-diphenylhydrazone, N-ethylcarbazole-N-methyl-N-phenylhydrazone, p-diethylaminobenzaldehyde-N- $\alpha$ -naphthyl-N-phenylhydrazone, p-diethylaminobenzaldehyde-3-methylbenzothiazolidinone-2-hydrazone, 2-methyl-4-N,N-diphenylamino- $\beta$ -phenylstilbene,  $\alpha$ -phenyl-4-N,N-diphenylaminostilbene and the like. Any of these resins can be used singly or in combination with other resins.

A photosensitive member thus formed may have an adhesion layer or a barrier layer between a substrate and a photosensitive layer. Suitable examples of materials contained in these layers are polyimide, polyamide, 25 nitrocellulose, polyvinyl butyral, polyvinyl alcohol, aluminium oxide and the like. It is preferable that the thickness of the layer is 1  $\mu$ m or less.

An azo compound of the invention is effective, in particular, as a charge generating material used in a 30 laminated-type photosensitive member. Working examples are shown below.

#### EXAMPLE 1

0.45 part by weight of the azo compound of the invention wherein A is



and the coupler is (1) component in the general formula (I), 0.45 part by weight of polyester resin (Vylon 200 made by TOYOB0) and 50 parts by weight of cyclohexanone were taken a Sand grinder for dispersion. The dispersion solution of the bisazo pigment was dispersed onto aluminotype-Mylar of 100  $\mu$ m in thickness by a 45 film applicator to form a charge generating layer so that a thickness of the dried layer is 0.3 g/m<sup>2</sup>. A solution of 70 parts of p-diphenylaminobenzaldehyde-N,N-diphenylhydrazone and 70 parts of polycarbonate resin (K-1300; made by TEIJIN KASEI) dissolved in 400 parts of dioxane was dispersed onto the above formed 50 charge generating layer to form a charge transporting layer so that the dried thickness of the layer is 16  $\mu$ m. Thus, a photosensitive member with the two layers 55 were prepared.

An exposure value for half-reducing ( $E_{\frac{1}{2}}$ ) obtained is in Table 1. The exposure value for half reducing, which is the exposure amount required for the surface potential to be half the value of the initial surface potential, is measured by first charging a photosensitive member by 65 means of a corona-discharge of -6.5 KV in the dark and then exposing the member to white light of 5 lux in illuminance.

#### EXAMPLES 2-4

Photosensitive members were prepared in a manner similar to EXAMPLE 1, except that the coupler components (6), (10), and (12) were used.

The results were shown in the Table 1.

#### EXAMPLES 5-8

Photosensitive members were prepared in a manner similar to EXAMPLE 1, except that azo components, wherein A was



and the coupler components were (2), (3), (7) and (26) in the general formula (I) were used.

The results are shown in Table 1.

TABLE 1

| example | A                                                                                    | coupler | $E_{\frac{1}{2}}$<br>(lux · sec) |
|---------|--------------------------------------------------------------------------------------|---------|----------------------------------|
| 1       |    | 1       | 4.5                              |
| 2       |    | 6       | 3.8                              |
| 3       |  | 10      | 3.1                              |
| 4       |  | 12      | 3.5                              |
| 5       |  | 2       | 3.0                              |
| 6       |  | 3       | 3.2                              |
| 7       |  | 7       | 2.7                              |
| 8       |  | 26      | 2.9                              |

#### EXAMPLES 9-12

Photosensitive members were prepared in a manner similar to EXAMPLE 1 except that  $\alpha$ -phenyl-4-N,N-diphenylaminostilbene was used as a charge transporting material and azo components, wherein A was:



and the preferred coupler components were (2), (14), (21) and (27) in the general formula (I) were used.

The results are shown in Table 2

#### EXAMPLES 13-16

Photosensitive members were prepared in a manner similar to EXAMPLE 1 except that azo components, wherein A was:

and the coupler components were (9), (11), (16) and (27) in the general formula (I) were used.

The results are shown in Table 2.

TABLE 2

| example | A | coupler | $E^{\frac{1}{2}}$<br>(lux · sec) |
|---------|---|---------|----------------------------------|
| 9       |   | 2       | 3.3                              |
| 10      |   | 14      | 2.7                              |
| 11      |   | 21      | 3.5                              |
| 12      |   | 27      | 2.4                              |
| 13      |   | 9       | 2.9                              |
| 14      |   | 11      | 2.6                              |
| 15      |   | 16      | 2.3                              |

TABLE 2-continued

| example | A | coupler | $E_{\frac{1}{2}}$<br>(lux · sec) |
|---------|---|---------|----------------------------------|
| 16      |   | 27      | 2.1                              |

## EXAMPLES 17-20

Photosensitive members were prepared in a manner similar to EXAMPLE 1 except that



was used as a charge transporting material instead of p-diphenylaminobenzaldehyde-N,N-diphenylhydrazone and azo components, wherein A was



TABLE 3

| example | A | coupler | $E_{\frac{1}{2}}$<br>(lux · sec) |
|---------|---|---------|----------------------------------|
| 17      |   | 1       | 3.0                              |
| 20      |   | 14      | 1.9                              |
| 18      |   | 19      | 2.4                              |
| 25      |   | 26      | 2.2                              |
| 30      |   | 28      | 2.2                              |

## COMPARATIVE EXAMPLE 1

35 A photosensitive member was prepared in a manner similar to EXAMPLE 1 except that the compound represented by the formula;



and the coupler components were (1), (14), (26) and (28) in the general formula (I) were used.

The results are shown in Table 3.

50 was used as a charge generating material was used.

$E_{\frac{1}{2}} = 10.2$  lux.sec.

## COMPARATIVE EXAMPLE 2

55 A photosensitive member was prepared in a manner similar to EXAMPLE 1 except that the compound represented by the formula;



was used as a charge generating material.

$E_1 = 6.3$  lux.sec.

What is claimed is:

1. A photosensitive member comprising a photosensitive layer on an electroconductive substrate, said photosensitive layer comprising an azo compound represented by the formula (I):



wherein A represents an aromatic hydrocarbon ring or a heterocyclic ring; R<sub>1</sub> and R<sub>2</sub> independently represent hydrogen, halogen, an alkyl, an aralkyl, a phenyl group, a condensed polycyclic ring or a condensed heterocyclic ring; or R<sub>1</sub> and R<sub>2</sub> combinedly form a cyclic ring; n represents an integer from 1 to 4.

2. A photosensitive member according to claim 1, wherein the photosensitive layer comprises a charge generating layer and a charge transporting layer, said charge generating layer comprising the azo compound represented by the formula (I).

3. A photosensitive member according to claim 2, wherein the charge transporting layer comprises a charge transportable compound selected from the group of hydrazone and stilbene.

4. A photosensitive member according to claim 2, wherein the charge generating layer comprises the azo compound dispersed in a binder.

5. A photosensitive member comprising a photosensitive layer on an electroconductive substrate, said photosensitive layer comprising an azo compound represented by the formula (I):

5

(I) 15

20

30

40

55



wherein A represents an aromatic hydrocarbon ring or a heterocyclic ring; R<sub>1</sub> and R<sub>2</sub> independently represent hydrogen, an alkyl, a phenyl or a condensed ring; n represents an integer from 1 to 4.

6. A photosensitive member according to claim 5, wherein said condensed ring comprises a 2- or 3-membered ring.

7. A photosensitive member according to claim 6, wherein said condensed ring is a member selected from the group consisting of a naphthalene ring, an anthracene ring, a fluorenone ring and an anthraquinone ring.

8. A photosensitive member according to claim 5, wherein the photosensitive layer comprises a charge generating layer and a charge transporting layer, said charge generating layer comprising the azo compound represented by the formula (I).

9. A photosensitive member according to claim 8, wherein the charge transporting layer comprises a charge transportable compound selected from hydrazone and stilbene.

10. A photosensitive member according to claim 8, wherein the charge generating layer comprises the azo compound dispersed in a binder.

11. A photosensitive member comprising a photosensitive layer on an electroconductive substrate, said photosensitive layer comprising an azo compound represented by the formula (I):



wherein A represents an aromatic hydrocarbon ring or a heterocyclic ring; R<sub>1</sub> and R<sub>2</sub> independently represent hydrogen, an alkyl, phenyl, phenyl substituted by alkyl, trifluoromethyl, methoxy, nitro, diphenylamino, F, or Cl a condensed ring or a condensed ring substituted by nitro or chloro; n represents an integer from 1 to 4.

\* \* \* \* \*